

C. MATLOCK.

PROCESS AND APPARATUS FOR PRODUCING CARBON BLACK.  
APPLICATION FILED MAR. 14, 1921.

1,438,542.

Patented Dec. 12, 1922.



Inventor  
*Chauncey Matlock,*

By *Chester H. Braselton,*

his Attorney

## UNITED STATES PATENT OFFICE.

CHAUNCEY MATLOCK, OF BROOKLYN, NEW YORK, ASSIGNOR TO MONROE-LOUISIANA CARBON COMPANY, OF MONROE, LOUISIANA, A CORPORATION OF DELAWARE.

## PROCESS AND APPARATUS FOR PRODUCING CARBON BLACK.

Application filed March 14, 1921. Serial No. 452,291.

To all whom it may concern:

Be it known that I, CHAUNCEY MATLOCK, a citizen of the United States, residing at 207 Park Place, Brooklyn, county of Kings, State of New York, have invented certain new and useful Improvements in Processes and Apparatus for Producing Carbon Black, of which I declare the following to be a full, clear, and exact description.

10 The present invention relates to the production of carbon black and more particularly to a process and apparatus for the production of carbon black by the partial combustion of hydrocarbon.

15 Carbon black has been customarily produced heretofore by burning natural gas or other gaseous hydrocarbons in a large number of small burners in such a manner that the outer part of the flame received sufficient 20 air for complete combustion while the inner portion of the flame was subjected to a dissociating temperature and insufficient air for complete combustion. Through the dissociation and partial combustion of the hydrocarbons in the interior of the flame a small 25 amount of free carbon, together with some incompletely dissociated hydrocarbons, was formed. This carbon was collected, and the further oxidation of the hydrocarbons and 30 destruction of the carbons thus formed, through the access of air through the upper part of the flames, was prevented by contacting and chilling the flames with a cooled plate or other cold surface on which the 35 flames were caused to impinge. The production of carbon black in this manner not only involved a large and expensive installation for the burning of the gases in quantities sufficient to permit of commercial operation 40 but the quality of the carbon produced was impaired by the presence of partly dissociated hydrocarbons of a tarry or oily nature formed in the interior of the flame and deposited on the chilled plates together with 45 the carbon produced. These deposits of tarry matters were further decomposed on the chilled plates by continued heating and formed a denser carbon having a lower coloring power, lower porosity and being otherwise undesirable for many purposes.

50 An object of the present invention is to provide an efficient process of producing carbon black of high quality.

Another object of the present invention is

to provide a process for the production of 55 a carbon black free from deposits of moisture or other condensates or impurities.

With these and other objects in view the invention consists in the process described in the following specification and defined in the 60 claims.

The various features of the invention are illustrated in the accompanying drawing which shows a view, partly in vertical section, of a preferred form of an apparatus 65 for carrying on the present invention.

In the present invention the hydrocarbons which are to be used for the production of the carbon black are burned in comparatively large flames in which a complete and 70 thorough mixture of air for the partial combustion of the hydrocarbons is permitted, and the degree of oxidation of the hydrocarbons is controlled by regulating the air supply and the temperature conditions 75 throughout the flame to break up or dissociate and partially oxidize all of the hydrocarbon and form a maximum of free carbon particles. To this end a regulated quantity of hydrocarbon gases is supplied to the lower 80 part of a closed combustion chamber or furnace through a number of burners and is mixed with a regulated supply of air which is forced into the furnace below the burners by means of a blower or other air 85 supply means. Upon passing upwardly in the furnace the air and gas are mixed and ignited and the hydrocarbons are dissociated and burned to form carbon and gaseous products of combustion. A body of hot 90 products of combustion is preferably maintained in the furnace and the combustion of the hydrocarbons takes place within and surrounded by this body of hot products of combustion, the air and hydrocarbons being 95 thoroughly mixed and the complete combustion of the carbon produced being avoided by limiting the air supply to the minimum required to dissociate the hydrocarbons and sustain combustion. Throughout the combustion the mixture of hydrocarbons and air is surrounded by hot gases and the combustion reaction is not effected by contact with cold surfaces or in any other manner which would check the complete dissociation of the 100 hydrocarbons.

As the burning gases reach the upper part of the combustion chamber the dissociation

- or breaking up and desired partial combustion of the hydrocarbons will have been completed and the hot gases and suspended carbon are thereupon rapidly removed and 5 quickly chilled to prevent any further heating, reoxidation or other modification of the carbon already formed. The chilling of the products of combustion and carbon is carried to a point at which the carbon may 10 be separated from the gaseous products of combustion but the temperature of the chilled products is always maintained above the dew point of water and other condensable products in the gaseous products of combustion. The carbon is separated from the cooled products of combustion by means of bag filters or other suitable means, the 15 temperature during this separation being of course maintained above the dew point. 20 Referring more particularly to the accompanying drawing, a regulated supply of gaseous hydrocarbons is admitted to a furnace 1 through a supply pipe 2 and a controlling valve 3 and is distributed 25 throughout the lower part of the furnace by burners 4. A regulated supply of air sufficient to affect only a partial combustion of the hydrocarbons is forced by means of a fan or blower 5 through a supply conduit 6 and controlling damper 7 into the furnace 1 at a short distance below the burners 4. As the air passes upwardly into contact with the streams of hydrocarbon gases issuing from the burners 4 it is permitted to 30 mix with the hydrocarbons and upon the completion of the mixture the gases are burned in the furnace at a short distance above the burners. A body or blanket 8 of hot or incandescent products of combustion 35 is preferably maintained in the furnace extending upwardly from a short distance above the burners 4 and the completion of the mixture of the gas and air and the combustion of the hydrocarbons takes place in 40 this body or blanket of hot gases. Through this manner of treatment the hydrocarbons are subjected in the body gases to a substantially uniform temperature throughout out of contact with cold surfaces or cold gases. 45 The dissociation and combustion of the hydrocarbons is therefore, not affected through a local chilling or cooling of the burned gases. 50 As the gases reach the upper part of the furnace the desired reaction will have been completed and the gases are therefore quickly withdrawn through an outlet pipe 10 by means of a fan 12 and are forced at a high velocity through a cooling pipe 14. 55 The pipe 14 is cooled by means of streams of water supplied from distributing or drip pipes 16 or by other suitable cooling means by which, a moderate and uniform chilling of the pipe may be attained. Through the 60 rapid passage of the gases and carbon

through the pipe 16 a uniform cooling of the gases is produced, which taken in connection with the velocity of the gases, hinders the settling and collection in the cooling pipe of deposits of carbon.

The temperature to which the gases are cooled is determined by means of a thermometer 18 in a pipe 20 leading from the cooling pipes 14 to a carbon separating device 22. The temperature to which the gases are cooled is indicated by the thermometer and is regulated by controlling the quantity of gases entering the pipe 10 by adjusting the opening of a damper 24 in the pipe 10 and by controlling the quantity 75 of water supplied through a control valve 26 to the distributing pipe 16. The temperature of the gases passing in contact with the thermometer 18 is adjusted so that it is slightly above the dew point for moisture and other condensable vapors produced in the combustion of the hydrocarbons and contained in the products of combustion. The dew point for any particular case may of course be determined in the usual manner by cooling the gases to a point at which a deposit of dew or any condensable product is produced. In case the dew point produced in the combustion of any particular hydrocarbon is a temperature above that 90 at which the carbon may be conveniently separated from the gaseous products of combustion, it may be lowered by admitting into the cooled, or partly cooled gases, a sufficient amount of air or other dry gas, 95 care being taken, however, not to bring the air into contact with the partly burned gases at a temperature high enough to bring about a secondary combustion.

The carbon may be separated from the 100 cooled gaseous products of combustion by any suitable separating apparatus but a bag filter of the type illustrated in the accompanying drawing is preferred. In this type of separating apparatus the gases entering the separator are caused to pass upwardly through inverted bags of muslin or other suitable material 28 the lower open ends of which are fastened to openings 30 in a horizontal partition 32 dividing the 110 separator 22. As the gases pass through the filter they are freed from the suspended particles of carbon and are withdrawn from the upper part of the separator through an outlet pipe 34, a fan 36 being preferably 115 provided to create a suction and draw the gases through the filter bags. When a deposit of carbon has been formed on the inner surface of the bags to such an extent as to hinder the passage of gases there- 120 through the carbon is detached from the bags by giving the upper part of the bags a circulatory movement. To this end the tops of the bags are supported by blocks 38 sus- 125 pended from a frame 40 which may be os- 130

cillated or given a circulatory movement by means of an eccentric shaft 42 and a crank 44. To assist in the removal of the deposits of carbon, chains 46 are suspended from 5 blocks 38 and as the blocks are given a circulatory movement the chains are thrown against the sides of the bags and assist to detach the carbon. The carbon detached from the bags drops into a hopper 46, forming the lower part of the separator 22, and 10 may be removed by withdrawing a slide 48 in an opening 50.

While only the preferred embodiment of 15 the invention has been described in this specification, it will be apparent that the form and type of carbon separating device may be modified and that other changes in the apparatus and modification of the process may be made without departing from 20 the broader features of the invention.

Having described the invention what is claimed as new is:

1. A process of producing carbon black which comprises burning hydrocarbons with 25 an amount of air sufficient to form a substantial amount of free carbon from said hydrocarbon, maintaining a uniform mixture of air and hydrocarbons and uniform temperature conditions throughout said 30 burning, removing the products of combustion and suspended carbon particles resulting from said combustion, cooling said gases and carbon, filtering said suspended carbon from said gases and maintaining said gases 35 above the dew point of condensable vapors in said gases throughout said treatment and said filtering.

2. A process of producing carbon black which comprises burning hydrocarbons with 40 an amount of air sufficient to form a substantial amount of carbon from said hydrocarbons, maintaining a uniform mixture of the air and hydrocarbons and uniform temperature conditions throughout said burning 45 and maintaining the temperature throughout said flame above the temperature at which substantial amounts of tarry substances tend to form, removing said gas and suspended carbon particles resulting 50 from said combustion, cooling said gases and carbon, filtering said suspended carbon from said gases and maintaining said gases 55 above the dew point of condensable vapors in said gases during said treatment and said filtering.

3. A process of producing carbon black which comprises burning a mixture of hydrocarbons with an amount of air insufficient to oxidize all of the carbon of said hydrocarbons, completing the partial combustion of 60 said hydrocarbons out of contact with cooling surfaces, withdrawing the products of combustion and carbon from said furnace, cooling said products of combustion 65 and carbon to a temperature above the dew

point of water vapor and condensable vapors in said gases and separating the carbon from the gaseous products of combustion while maintaining the temperature of said products of combustion above said dew 70 point during the separation of said carbon from said gaseous products of combustion.

4. A process of producing carbon black which comprises burning a mixture of hydrocarbons and an amount of air insufficient 75 to completely oxidize said hydrocarbons, completing the partial combustion of said hydrocarbons out of contact with a cooling surface, withdrawing the products of combustion and carbon, cooling said products 80 of combustion and carbon to a temperature above the dew point of water and condensable vapors in said gases, filtering the carbon from the gaseous products of combustion and maintaining the temperature of 85 said products of combustion above said dew point during the filtration of said carbon from said gaseous products of combustion.

5. A process of producing carbon black which comprises partially oxidizing hydrocarbons to form suspended particles of free carbon, withdrawing said carbon suspended in the gaseous products of combustion, cooling said gases and said carbon to a point somewhat above the dew point of condensable vapors in said gases and separating the carbon from the cooled gases. 90

6. A process of producing carbon black which comprises maintaining a body of hot 100 products of combustion, introducing into said mass of products of combustion hydrocarbons and air in insufficient quantities to completely oxidize said hydrocarbons, said air and hydrocarbons being in intimate contact, effecting the partial combustion of 105 said hydrocarbons in said hot products of combustion, withdrawing the gases and carbon resulting from said combustion, cooling said products of combustion and carbon to a temperature above the dew point of condensable vapors in said products of combustion and separating said carbon from said gaseous products of combustion while maintaining the temperature of said products 110 above said dew point. 115

7. A process of producing carbon black which comprises effecting the partial combustion of hydrocarbons in an atmosphere of hot products of combustion, withdrawing hot products of combustion and suspended carbon, cooling said products of combustion and carbon to a temperature but slightly above the dew point of said products of combustion and separating said carbon from the gaseous products of combustion while maintaining said products of combustion and carbon at a temperature 120 above said dew point. 125

8. A process of producing carbon black which comprises burning hydrocarbons with 130

air sufficient to only partially oxidize all of said hydrocarbons and to form free carbon, completing the uniform partial oxidation of said hydrocarbons by said insufficient quantity of air, thereafter chilling said products of combustion to a temperature at which the carbon may be conveniently fil-

tered or otherwise separated from the hot gases without precipitating moisture or oils and separating said carbon from said gases 10 at said temperature.

In testimony whereof I affix my signature.

CHAUNCEY MATLOCK.